

Jan. 16, 1951

M. E. NASH

2,538,321

## TREATMENT OF LUBRICATING OILS

Filed Sept. 8, 1947



## UNITED STATES PATENT OFFICE

2,538,321

## TREATMENT OF LUBRICATING OILS

Martin E. Nash, Bartlesville, Okla., assignor to  
Phillips Petroleum Company, a corporation of  
Delaware

Application September 8, 1947, Serial No. 772,877

7 Claims. (Cl. 196—14.19)

1

This invention relates to the treatment of lubricating oils to improve their properties. In one of its more specific aspects it relates to a treatment of a lubricating oil which increases its viscosity or viscosity index, and otherwise improves various properties.

Lubricating oil as referred to herein includes all such products, and their base stocks, which have a viscosity of about 32 SUS (Saybolt Universal Seconds) at 210° F. to about 350 SUS at 210° F., and as are usually understood to be covered by this term by those skilled in the art. It includes particularly lubricating oil stocks, such as a paraffin-base stock, a naphthalene-base stock, a mixed-base stock, or a synthetic-base stock, which are refined for use as engine lubricants. By blending these " neutrals" and " bright stocks" engine lubricating oils of varying viscosity indices are produced.

Lubricating oils of high quality have been manufactured by many processes including sulfuric acid refining, aluminum chloride refining, solvent refining, and hydrofluoric acid refining. The sulfuric acid process improves some of the properties of the oil but in doing so a large portion of the acid is consumed in the process and is not economically recoverable. The sulfuric acid-sulfur dioxide process has the same disadvantage, in that a greater part of the acid is nonrecoverable, making the process overly expensive. Solvent refining processes are known in the prior art using sulfur dioxide. They also improve some of the properties of the lubricating oil, but also leave objectionable sulfur compounds. Hydrofluoric acid refining as shown in the prior art improves some properties of lubricating oil by removing gum-forming compounds, olefins, and at relatively low pressure small amounts of aromatics, and may promote alkylation between some of the compounds which are usually present.

Broadly speaking, my invention comprises a process of improving lubricating oil by contacting the lubricating oil with substantially anhydrous hydrofluoric acid and sulfur dioxide. In a preferred modification, this initial treatment is followed by a further treatment with substantially anhydrous hydrofluoric acid, recovering the lubricating oil from the resulting mixture.

In accordance with this invention, lubricating oil is substantially improved by treating with a mixture of anhydrous hydrofluoric acid, and sulfur dioxide, without the numerous disadvantages which generally accompany the use of these reagents when employed singly. Olefins, aromatics,

2

unsaturated resins, gum-forming bodies, and other undesirable components are removed by the hydrofluoric acid-sulfur dioxide mixture. An added advantage of the hydrofluoric acid-sulfur dioxide treatment is the recovery by solvent extraction of the sulfur dioxide which is usually lost when used alone or in other combinations, and by inhibiting the formation of undesirable sulfur compounds. If desired, a light hydrocarbon may be used as a diluent for the oil during treatment, such diluent generally being a readily liquefiable paraffin such as liquid propane, etc.

In a preferred embodiment of this invention, the treated oil is subsequently contacted with substantially anhydrous hydrofluoric acid to remove any residual undesired sulfur compounds.

An object of the present invention is to provide a novel and improved method of improving lubricating oils. Another object is to provide a method of improving natural lubricating oils. A further object is to provide a method of improving mixed-base lubricating oils. Another object is to provide a method of improving the viscosity index of natural or synthetic lubricating oils. Other objects and advantages of this invention will become apparent from the accompanying disclosure and discussion.

The accompanying drawings illustrate diagrammatically two embodiments of apparatus for the practice of the present invention.

A most important improvement in the oils treated by the present process is in the viscosity index which is determined by the method described in an article entitled Viscosity Variations of Oils With Temperatures, by E. W. Dean and G. H. G. Davis, in Chemical and Metallurgical Engineering, volume 36, page 619 (1929). The viscosity index of a lubricating oil is an indication of its composition or type, i. e., whether it is a paraffin-base or naphthalene-base oil. Paraffin-base oils have high viscosity indices, naphthalene-base oils have relatively low viscosity indices, and mixed-base oils have viscosity indices between these extremes. This index is likewise a measure of the ability of a lubricating oil to remain viscous at high temperatures. As is well known, oils lose their viscosity rapidly with an increase in temperature. The oil with a high viscosity index will, however, lose its viscosity less rapidly than an oil with a low viscosity index when the temperature is increased, or conversely, will not have its viscosity unduly increased by a lowering of temperature. The present invention increases this viscosity index and may also increase the absolute viscosity at the standard 210° F. temperature for measurement of viscosity.

Any suitable equipment may be employed for the performance of the present invention, and equipment which is resistant to the corrosive action of hydrofluoric acid is particularly desirable. Conventional contacting equipment similar to contactors which are commonly used for conducting the alkylation of isoparaffins with olefins may be used to provide suitable contact between the reactants. Any other means of maintaining an intimate contact of the lubricating oil and acid phases may be employed. The equipment should be provided with means for maintaining the desired temperatures and pressures in the various zones.

The temperature range necessary for the practice of this invention is from about -20° to about 50° F. The pressure is not critical, but sufficient pressure is preferably used to maintain all reactants in liquid phase. The reactants should be contacted for a sufficient length of time for the improvement of the oil to take place. The treating time for the oil, hydrofluoric acid, and sulfur dioxide mixture is about 30 to about 300 minutes, and for the oil and hydrofluoric acid mixture is about 5 to about 30 minutes.

In the performance of one embodiment of the present invention, a lubricating oil may be treated according to the process described above, allowed to separate, usually by gravity, into two separate layers, namely the lower layer or acid phase and the upper layer or hydrocarbon phase. A portion of the lower layer or acid phase is recycled to the initial contactor and the remainder is passed to a fractionator where the hydrofluoric acid and sulfur dioxide are recovered. The upper layer or hydrocarbon phase is passed to an extractor where it is treated with hydrofluoric acid.

In the performance of the second embodiment of the present invention, a lubricating oil may be treated, according to the process described, in an initial contact zone with a mixture of substantially anhydrous hydrofluoric acid and sulfur dioxide and in a second contact zone with hydrofluoric acid alone. The treated oil is then fractionated and the hydrofluoric acid-sulfur dioxide mixture removed for further fractionation.

In either of the above embodiments of this invention, if desired, the hydrofluoric acid and sulfur dioxide may be introduced to the contactor separately, however, the preferred method is to mix the acid and sulfur dioxide prior to introduction to the contactor.

The hydrofluoric acid and sulfur dioxide used in the practice of this invention can be of the quality of the commercial products. The hydrofluoric acid referred to as anhydrous hydrofluoric acid is commercial anhydrous hydrofluoric acid, and those skilled in the art know it may contain small amounts of sulfur dioxide (usually less than 1 weight per cent), water, and other impurities.

The process may be carried out either in a batchwise manner or continuously, the latter being preferred for commercial operation. A better understanding of this invention may be had by reference to the accompanying drawings which illustrate, by means of a diagrammatic flow sheet, an over-all process of a preferred embodiment of the present invention.

As shown in Figure 1 lubricating oil is introduced through line 10 to a contactor 11, the hydrofluoric acid and sulfur dioxide mixture in the weight ratio of sulfur dioxide to hydrofluoric acid of about 1:3 to about 3:1 is introduced to contactor 11 through line 12, and a low boiling paraffinic diluent such as isopentane is introduced

through line 13, valve 14, and line 10. The range of ratios of oil to hydrofluoric acid-sulfur dioxide is from 1:5 to 5:1, depending on the properties of the material to be treated. The four components are intimately mixed in contactor 11 for a suitable reaction period and the effluent passed through line 15 and valve 16 to settler 17 in which separate an upper or hydrocarbon-rich layer and a lower layer rich in hydrofluoric acid and sulfur dioxide. At least a portion of the lower layer may be recycled through line 19 and valve 20 to contactor 11; the remainder is passed through line 21 and valve 22 to fractionator 38. In fractionator 38 the acid-sulfur dioxide mixture is fractionated to yield a high-boiling organic material which is removed through line 39 and valve 40; a hydrofluoric acid-water azeotrope, removed through line 41 and valve 42; and a hydrofluoric acid-sulfur dioxide fraction, removed through line 43 and valve 44 to fractionator 45. The hydrofluoric acid and sulfur dioxide are separated in fractionator 45, the sulfur dioxide removed overhead through line 12 and valve 47, and anhydrous hydrofluoric acid removed as a bottoms product through line 49 and valve 50. A portion of the hydrofluoric acid stream carried through line 49 is passed to line 12 through line 51 and valve 52, and a mixture of hydrofluoric acid and sulfur dioxide thus recycled to contactor 11 via line 12, thence following a previously described route. The remaining hydrofluoric acid carried in line 49 is introduced to extractor 23 through valve 24, following a route subsequently described. Make-up hydrofluoric acid may be added to line 49 through line 53 and valve 54, and make-up sulfur dioxide may be added through line 55 and valve 56 to line 12.

The upper layer obtained in settler 17 is passed through line 25 and valve 26 to extractor 23 in which it is countercurrently contacted with hydrofluoric acid which enters through line 49. Hydrofluoric acid withdrawn from extractor 23 is passed through line 27, valve 28, and line 19 to contactor 11. In extractor 23 undesired sulfur compounds remaining in the oil are extracted by the hydrofluoric acid. In some cases, especially when contactor 11 is maintained substantially above 20° C. it is advantageous to maintain extractor 23 at a lower temperature, e. g., about -20° to about 0° C., in order to improve the color of the oil. Furthermore, in some cases the hydrofluoric acid entering through line 49 may constitute all the acid charged to the contactor and the material charged through line 12 may be substantially pure sulfur dioxide. In this mode of operation, valve 52 is closed.

Extracted hydrocarbon effluent from extractor 23 is passed through line 29 and valve 30 to fractionator 31, which may be operated at sub-atmospheric pressure if desired. An overhead fraction comprising chiefly low-boiling paraffin and hydrofluoric acid is withdrawn from fractionator 31 through lines 32 and valve 33 and recycled to contactor 11. A kettle product having a boiling range similar to the untreated oil is withdrawn through line 34 and valve 35 as the main product of this process. This oil may be further treated by such conventional methods as alkali washing, clay treating, etc., as desired.

The contactor described in Figure 2 as a second embodiment of this invention takes the place of contactor 11, settler 17, and extractor 23. Where the same identification numerals are used in both

Figures 1 and 2 they represent the same apparatus. As shown in Figure 2, the oil to be treated enters liquid-liquid contactor 60 through line 10, having previously been diluted with a low-boiling paraffin if desired. Contactor 60 may be provided with such internal members as perforated plates, packing, baffles, etc., to facilitate contacting. The oil rises through contactor 60 and contacts a downward-flowing liquid mixture of hydrofluoric acid and sulfur dioxide in the lower zone. A mixture of hydrofluoric acid and sulfur dioxide or, if desired, sulfur dioxide alone, enters contactor 60 through intermediate inlet 12. After contact with the hydrofluoric acid-sulfur dioxide mixture in the lower zone, the oil is contacted in the upper zone with hydrofluoric acid alone, which enters through upper inlet 49. The treated oil is withdrawn through outlet 29 to fractionator 31, of Figure 1, and treated as previously described for removal of dissolved hydrofluoric acid and light paraffin. A mixture of hydrofluoric acid and sulfur dioxide is withdrawn through outlet 19 and is recycled to contactor 60, Figure 2, and/or distilled as in the previously described embodiment. The flow rates of the liquid entering contactor 60 through inlets 12 and 49, are so interrelated that the composition of the downward-flowing mixture in the lower zone of the contactor is within the range previously specified.

Various additional valves, pumps, and other conventional equipment necessary for the successful practice of this invention will be familiar to one skilled in the art and have been omitted from these schematic drawings for sake of clarity.

Following are specific examples of the treatment of lubricating oil with a mixture of hydrofluoric acid and sulfur dioxide in the presence of a low-boiling paraffin solvent.

#### Example I

A mixture of 880 grams of lubricating oil, 627 grams of anhydrous hydrofluoric acid, 632 grams of isopentane, and 418 grams of sulfur dioxide was shaken in a Monel bomb for two hours at room temperatures by means of a rocker mechanism. The bomb was removed from the rocker and allowed to stand in a vertical position for one hour, after which the hydrofluoric acid-sulfur dioxide layer was removed. The treated oil-isopentane mixture was then washed with dilute sodium hydroxide and filtered through Hyflo Super-Cel. The filtered oil was topped under vacuum to the initial boiling range of the original oil. The properties of the product oil were determined by conventional methods. The following results were obtained.

|                                                    | Untreated<br>Oil A | Treated<br>Oil A |
|----------------------------------------------------|--------------------|------------------|
| Viscosity at:                                      |                    |                  |
| 100° F. SUS                                        | 343.9              | 333.9            |
| 210° F. SUS                                        | 53.39              | 53.36            |
| Viscosity index                                    | 85.9               | 90.0             |
| Pour point, F.                                     | 15                 | 15               |
| ASTM color                                         | 24                 | 4                |
| API gravity                                        | 28.3               | 29.1             |
| Refractive index at 20° C.                         | 1.4893             | 1.4866           |
| Aluminum block stability data:                     |                    |                  |
| Neutralization No.:                                |                    |                  |
| Before heating                                     | 0.00               | 0.02             |
| After heating                                      | 0.33               | 0.22             |
| Ramsbottom C res., wt. per cent—                   |                    |                  |
| Before heating                                     | 0.02               | 0.04             |
| After heating                                      | 0.21               | 0.19             |
| Naphtha insolubles after heating, wt. per cent     | 0.08               | 0.02             |
| Evaporation loss, wt. per cent                     | 4.3                | 3.2              |
| Viscosity increase corr. for evapn. loss, per cent | 5.2                | 4.4              |

#### Example II

A mixture of 878 grams of a lubricating oil similar to that used in Example I, 922 grams of anhydrous hydrofluoric acid, and 620 grams of isopentane was shaken in a Monel bomb at room temperature for two hours by means of a rocker mechanism. The bomb was removed from the rocker and allowed to stand in a vertical position for one hour, after which the hydrofluoric acid layer was removed. The treated oil-isopentane mixture was then washed with dilute sodium hydroxide and filtered through Hyflo Super-Cel. The filtered oil was topped under vacuum to the initial boiling range of the original oil. The properties of the product oil were determined by conventional methods. The following results were obtained.

|                                                    | Untreated<br>Oil B | Treated<br>Oil B |
|----------------------------------------------------|--------------------|------------------|
| Viscosity at:                                      |                    |                  |
| 100° F. SUS                                        | 287.3              | 288.7            |
| 210° F. SUS                                        | 50.77              | 50.86            |
| Viscosity index                                    | 89.1               | 89.4             |
| Pour point, F.                                     | 30                 | 25               |
| ASTM color                                         | 23                 | 2                |
| API gravity                                        | 28.7               | 29.0             |
| Refractive index at 20° C.                         | 1.4879             | 1.4863           |
| Aluminum block stability data:                     |                    |                  |
| Neutralization No.:                                |                    |                  |
| Before heating                                     | 0.00               | 0.02             |
| After heating                                      | 0.33               | 0.22             |
| Ramsbottom C res., wt. per cent—                   |                    |                  |
| Before heating                                     | 0.02               | 0.04             |
| After heating                                      | 0.21               | 0.19             |
| Naphtha insolubles after heating, wt. per cent     | 0.08               | 0.02             |
| Evaporation loss, wt. per cent                     | 4.3                | 3.2              |
| Viscosity increase corr. for evapn. loss, per cent | 5.2                | 4.4              |

The data from Example I show that a substantial increase in viscosity index is obtained by treatment with hydrofluoric acid and sulfur dioxide. The high neutralization number before heating (2.96) is due to the presence of unstable sulfur compounds, and may be lowered by a subsequent treatment with hydrofluoric acid alone. The ASTM color may also be lowered in this manner.

Comparison of the data from Example II with that of Example I indicates the beneficial effects of treatment with mixtures of hydrofluoric acid and sulfur dioxide. When sulfur dioxide was present the increase in viscosity index was about 5 per cent, whereas, when sulfur dioxide was absent the increase was only about 0.3 per cent.

Although the process has been described and exemplified in terms of its preferred modifications, it is understood that various changes may be made without departing from the spirit of the process as disclosed and expressed in the claims.

#### I claim:

1. A process of manufacturing a lubricating oil of improved properties which comprises thoroughly agitating a lubricating oil with a mixture of anhydrous hydrofluoric acid and sulfur dioxide, containing about 25 to 75 weight per cent sulfur dioxide, in the ratio of oil to treating mixture of about 1:5 to about 5:1, at sufficient pressure to maintain the hydrofluoric acid and sulfur dioxide substantially liquid, and at a temperature between about -20° and about 50° C., and for about 30 to about 300 minutes.
2. A process of manufacturing a lubricating oil of improved properties which comprises thoroughly agitating a lubricating oil with a mixture of substantially anhydrous hydrofluoric acid and sulfur dioxide, containing about 25 to 75 weight

per cent sulfur dioxide, in the ratio of oil to treating mixture of about 1:5 to about 5:1, and further extracting said oil with substantially anhydrous hydrofluoric acid in the ratio of oil to hydrofluoric acid of about 1:5 to about 5:1, at sufficient pressure to maintain the hydrofluoric acid and sulfur dioxide substantially liquid, and at a temperature between about -20° and about 50° C., and for about 30 to about 300 minutes.

3. A process of manufacturing a lubricating oil of improved viscosity index which comprises treating a lubricating oil in an initial contact zone with substantially anhydrous hydrofluoric acid and sulfur dioxide, separating the treated mixture into an acid phase and a hydrocarbon phase, separating said acid phase into a heavy hydrocarbon fraction, a hydrofluoric acid-water azeotrope fraction, and a hydrofluoric acid-sulfur dioxide fraction, separating said acid-sulfur dioxide fraction into hydrofluoric acid and sulfur dioxide for recycle, recycling at least a portion of said separated hydrofluoric acid and sulfur dioxide to said initial contact zone, and fractionating said hydrocarbon phase recovering said improved lubricating oil.

4. A process of manufacturing a lubricating oil of improved viscosity index which comprises treating a lubricating oil in an initial contact zone with substantially anhydrous hydrofluoric acid and sulfur dioxide, separating the treated mixture into an acid phase and a hydrocarbon phase, separating said acid phase into a heavy hydrocarbon fraction, a hydrofluoric acid-water azeotrope fraction, and a hydrofluoric acid-sulfur dioxide fraction, separating said acid-sulfur dioxide fraction into hydrofluoric acid and sulfur dioxide for recycle, recycling said separated sulfur dioxide to said initial contact zone and at least a portion of said separated hydrofluoric acid to a subsequently described hydrocarbon extraction zone, contacting countercurrently said hydrocarbon phase with hydrofluoric acid in an extraction zone, recycling said acid after contact with said hydrocarbon phase to said initial contact zone, fractionating the resulting extracted hydrocarbon and recovering said improved lubricating oil.

5. A process of manufacturing a lubricating oil of improved viscosity index which comprises treating a lubricating oil in an initial contact

zone with substantially anhydrous hydrofluoric acid and sulfur dioxide, and further treating said oil in a second contact zone with substantially anhydrous hydrofluoric acid, separating the treated mixture into an acid phase and a hydrocarbon phase, separating the hydrofluoric acid from said acid phase, recycling at least a portion of said separated hydrofluoric acid, fractionating said hydrocarbon phase, and recovering said improved lubricating oil.

6. A process of manufacturing a lubricating oil of improved viscosity index which comprises thoroughly agitating a lubricating oil with a mixture of substantially anhydrous hydrofluoric acid and sulfur dioxide, in the volume ratio of oil to treating mixture of about 1:1, for about 30 to about 300 minutes, at sufficient pressure to maintain the hydrofluoric acid and sulfur dioxide substantially liquid, at a temperature between about 20 and about 30° C., and recovering the said improved lubricating oil as a product of the process.

7. A process of manufacturing a lubricating oil of improved viscosity index which comprises thoroughly agitating a lubricating oil with a mixture of substantially anhydrous hydrofluoric acid and sulfur dioxide, in the volume ratio of oil to treating mixture of about 1:1, for about 30 to about 300 minutes, at sufficient pressure to maintain the hydrofluoric acid and sulfur dioxide substantially liquid, and at a temperature between about 20 and about 30° C.; further extracting with liquid substantially anhydrous hydrofluoric acid in the volume ratio of oil to hydrofluoric acid of about 1:1, for about 5 to about 30 minutes, at a temperature between about 20 and about 30° C., and recovering the said improved lubricating oil as a product of the process.

MARTIN E. NASH.

40

#### REFERENCES CITED

The following references are of record in the file of this patent:

45

#### UNITED STATES PATENTS

| Number    | Name           | Date          |
|-----------|----------------|---------------|
| 2,378,762 | Frey           | June 19, 1945 |
| 2,438,565 | Linn et al.    | Mar. 30, 1948 |
| 2,440,258 | Elliott et al. | Apr. 27, 1948 |

50